

## UNITED STATES PATENT OFFICE

2,379,429

## ALLOY FOR USE IN ELECTROLYTIC CELL

Donald W. Forsgren and Waldo W. Forsgren,  
Salt Lake City, Utah, assignors to U. S. Metallic  
Magnesium Company, Salt Lake City, Utah

No Drawing. Application September 17, 1943,  
Serial No. 502,827

1 Claim. (Cl. 75—169)

Our invention relates to the reduction of and production of magnesium metal utilizing an alloy of lead, bismuth, and mercury as an inter-phase in the direct reduction of magnesium from brines and the like in electrolytic cells as already set out by us in our copending application for patent, Serial No. 454,278, filed August 10, 1942, in which we disclosed the use of mercury as the inter-phase medium. The benefits derived from this particular amalgam is that the amalgam has a lower surface tension than that of the system formerly used of mercury and magnesium. When the scum which usually and ordinarily forms on mercury in an electrolytic cell and which is chiefly a compound  $MgHg_2$  forms on the alloy, containing mercury, lead, and bismuth, it is not retarding to the action as this alloy having a lower

surface tension, permits or causes the surface scum to be drawn inwardly toward the worm or agitator of the cell in which it is used passing through the cell freely thereby increasing the efficiency of the cell and consequently the production of the magnesium metal.

The alloy consists of 12.4% lead; 13.02% of bismuth, and the balance of mercury.

Having thus described our invention we desire to secure by Letters Patent and claim:

A new alloy for use in electrolytic cells for use in the production of magnesium metal comprising 12.4% lead, 13.02% bismuth and 74.58% mercury.

DONALD W. FORSGREN.  
WALDO W. FORSGREN.